

Nov. 3, 1936.

W. C. DEVEREUX ET AL

2,059,984

TREATMENT OF NONFERROUS ALLOY CASTINGS

Filed Dec. 12, 1934



Inventors  
Wallace C. Devereux &  
Christopher S. Oliver

by *Ernest J. Meekin*  
Their Attorney

Patented Nov. 3, 1936

2,059,984

# UNITED STATES PATENT OFFICE

2,059,984

## TREATMENT OF NONFERROUS ALLOY CASTINGS

Wallace Charles Devereux, Slough, and Christopher Sibley Oliver, Coventry, England, assignors, by mesne assignments, to The Dow Chemical Company, Midland, Mich., a corporation of Michigan

Application December 12, 1934, Serial No. 757,204  
In Great Britain June 18, 1934

10 Claims. (Cl. 148—4)

This invention relates to the treatment of non-ferrous alloy castings with more especial reference to the treatment of castings composed of magnesium alloys which castings, in spite of the most rigorous control and attention during the casting operation are inclined to exhibit some permeability under the rigorous tests applied to articles of this character and in the manufacture of which accordingly there has hitherto been a large number of rejections.

The present invention has for its object to provide an inexpensive process for the treatment of alloy castings which effectively removes permeability without necessarily modifying the surface appearance or affecting the inherent structure of the casting and by which the number of rejected castings may be substantially reduced or even eliminated.

In accordance with the present invention alloy castings are impregnated with a readily fusible alloy having a low viscosity when in fluid condition so as to be capable of penetrating to the inter-crystalline crevices in the structure of the casting and adapted on solidification to unite with the parent alloy and thereby render the structure impermeable under pressure.

In selecting the fusible alloy for the impregnating treatment it is desirable, if not necessary, to have regard to the contraction characteristics on cooling, since if the coefficient of contraction of the fusible alloy is such that on solidification and cooling it contracts to a greater extent than the parent casting, voids are likely to occur in the casting, and the object of the process will be defeated.

Further, it is desirable to employ as the impregnating alloy some eutectic mixture which will further alloy or amalgamate with the parent casting on solidification and subsequently in such manner that by the amalgamation the characteristics of the inserted material are altered, for instance by a material elevation of the melting point, thereby to guarantee effective union under working condition.

To this end the constitution of the impregnating alloy may vary according to the constitution of the alloy from which the casting to be treated is manufactured, and in general alloys will be utilized which are fusible at temperatures below 100° C., whereby impregnation can be effected without recourse to unduly high temperatures and without likelihood of distorting the castings.

As aforementioned, castings of magnesium alloys present a greater inclination to weep than do castings of aluminium alloys or other kindred materials, and for the impregnation of such magnesium alloy castings an alloy composed of tin, lead, bismuth and cadmium having a melting point of approximately 68.05° C. has been found especially suitable.

In the practice of the invention, an impregnating alloy of sufficiently low melting point is obtained by employing a fusible alloy containing bismuth, lead and tin, while if a melting point below 75° C. is required a cadmium component may be added. Wood's metal is suitable for the purpose, although, preferably, the bismuth content of the fusible alloy used for impregnation, while not being less than 40%, is present in substantially this proportion and consequently is a lower proportion than in Wood's metal.

Applying the process according to the invention to a magnesium alloy casting, the casting is heated to and maintained at a temperature in the vicinity of 160° C. in any appropriate manner during the treatment, and the impregnating alloy, previously heated to a temperature of 80° C., is run into or on to the casting and is forced therethrough by the application of sufficient pressure. It has been found that excessive pressure is not called for owing to the fluidity and penetrating power of the molten alloy which, under the conditions of treatment, impregnates the casting and weeps freely from the opposite surface thereof.

The surface adhesion between the impregnating alloy and the parent structure is, however, negligible, and, at the conclusion of the treatment, the surface of the casting does not exhibit any trace of the impregnation to which it has been subjected.

On the other hand, castings which exhibit a pronounced tendency to weep under pressure prior to impregnation prove effectively impermeable after the treatment even under temperature conditions considerably above the melting point of the fusible alloy which would seem to show that on solidification the fusible alloy unites with and forms an integral part of the metallic structure of the casting.

The invention will be further described with reference to the accompanying explanatory drawing which illustrates by way of example one form of apparatus for carrying the process into effect, and in which the numeral 1 generally designates the article composed of magnesium alloy which it is desired to render impermeable, in the case illustrated, the rear crank-case cover of a radial aircraft engine.

In the first place, any apertures, there being five in the casting illustrated, are effectively blocked by means of removable clamp plates or solid washers 2 faced with appropriate heat resistant packing material 3 such as Hallite.

To the most convenient aperture, the lower end of a plunger or ram cylinder 4 is secured, either with or without packing material, by means of clamping rods 5 passing over the base 6 of such cylinder 4 around the casting 1, and being securely attached to a pedestal or machine bed 7.

The assembly including the casting 1, plunger cylinder 4 and bed 7 are then heated in an electric furnace or in other appropriate manner to a temperature of about 160° C., and meanwhile the impregnating alloy is melted.

5 After the casting has been heated sufficiently to attain a temperature of 160° C. throughout, the assembly is withdrawn from the furnace and placed in a press in such manner as to leave its major surface area exposed, whereafter the fused alloy is poured through the ram cylinder until the interior of the casting is filled.

10 Thereupon the ram or plunger, designated 8, is replaced in its cylinder and the press closed to 15 apply pressure through it to the body of liquid alloy located in the casting.

Under light pressures the fusible alloy impregnates the casting and weeps freely from its outer face as a fine and substantially invisible mist or spray which, as it is cooled by the atmosphere, sublimes or solidifies on the bed as a soft metallic wool.

20 The process is continued for a period depending on the form and shape of the casting—usually for about five minutes—additional quantities of fusible alloy being inserted in the cylinder 4, if required, and while the casting is still above the melting temperature of the fusible alloy the clamps 8 are removed and the molten alloy 25 poured from the interior of the casting 1 into an appropriate container for subsequent use in the next treatment.

30 The casting is then permitted to cool, and, during cooling, it will be noticed that the sweating continues, beads of the fusible alloy forming on the surface of the casting, this being the result of the difference of contraction on cooling between the parent casting and the fusible alloy; in fact, it has been established that the particular fusible alloy preferred for use with magnesium castings and composed of bismuth, lead, tin and cadmium, actually expands on solidifying and cooling, an approximate figure for the cubical expansion in solidifying from the melting temperature and cooling to 20° C. being 0.243%.

35 The treated casting is then permitted to set, being left preferably for some days, during which period amalgamation between the fusible alloy and that of the parent casting takes place, this being corroborated by the fact that where a treated casting has been cured and attempt is made again to subject it to the process according to the invention, it is found to be impermeable to the fusible alloy under pressure, from which the conclusion may be drawn that the fusible alloy inserted into the casting during the original treatment has amalgamated with the parent structure to form an alloy of different composition, having a considerably higher melting point.

40 It should be noted that the quantity of fusible alloy used in the impregnating treatment is negligible, the difference in mass of the casting before and after treatment being almost imperceptible, the illustrated casting weighing 2 lbs. 8 ozs. 2 drams prior to treatment, and after treatment gaining only 3 drams, or approximately .78%.

45 The proportions of the constituents would not appear to be critical, most satisfactory results having been obtained with bismuth, lead, tin and cadmium in the proportions of 42%, 24.5%, 23% and 10.5% respectively on castings of magnesium alloyed with aluminum, copper, zinc, cadmium and/or manganese.

The particular apparatus illustrated is especially suited for applying the treatment to hollow castings such as pump casings and crank cases, e. g. for aero engines, but for other articles recourse may be had to a heated vat or tank with 5 which is associated evacuating mechanism, the casting being placed in the vat or tank which is then evacuated and filled with fusible alloy under pressure, thereby to effect impregnation, the pressure being subsequently released and the impregnated casting removed and permitted to cool.

10 By the treatment according to the present invention castings are rendered substantially impermeable and consequently the number of rejected castings is substantially reduced.

15 What we claim is:—

1. A process for the treatment of magnesium alloy castings to render them impermeable, consisting in heating the castings to a temperature of about 160° C. throughout, forcing thereinto 20 a fused alloy of bismuth, lead, tin and cadmium, while maintaining the temperature of the casting above the melting point of the fused alloy, and allowing the casting to cool and to amalgamate with the fused alloy on solidification. 25

2. In a process for the treatment of porous non-ferrous alloy castings comprising impregnating the castings with an alloy having a low melting point and a low viscosity when in fluid condition, the steps which consist in heating the 30 casting throughout to a temperature considerably above the melting point of the impregnating alloy and maintaining it above such melting temperature while forcing the impregnating alloy through the material of the casting under 35 pressure.

3. A process according to claim 2 in which the impregnating alloy employed is composed substantially of bismuth, lead and tin, such alloy being fusible at temperatures below 100° C. 40

4. A process according to claim 2 in which the impregnating alloy employed is composed substantially of bismuth, lead, tin and cadmium, such alloy being fusible at temperatures below 75° C. 45

5. A process for impregnating porous magnesium alloy castings to render the same impermeable which comprises forcing under pressure a molten alloy of low melting point and low viscosity when in fluid condition into the voids 50 in the material of such casting, while maintaining the temperature of the casting above the melting point of the fused alloy, and allowing the treated casting to cool.

6. A process according to claim 5 in which the impregnating alloy employed is composed substantially of bismuth, lead and tin, such alloy being fusible below 100° C. 55

7. A process according to claim 5 in which the impregnating alloy employed is composed substantially of bismuth, lead, tin and cadmium, such alloy being fusible below 75° C. 60

8. A process according to claim 5 in which the impregnating alloy employed is composed of approximately 42 per cent bismuth, 24.5 per cent 65 lead, 23 per cent tin, and 10.5 per cent cadmium.

9. Non-ferrous alloy castings rendered impermeable by treatment according to the process defined in claim 2.

10. Magnesium alloy castings rendered impermeable by treatment according to the process defined in claim 5. 70

WALLACE CHARLES DEVEREUX.  
CHRISTOPHER SIBLEY OLIVER.